

R. G. MILLER.

VITREOUS WARE AND METAL AND METHOD OF MAKING SAME.  
APPLICATION FILED APR. 12, 1911.

1,164,840.

Patented Dec. 21, 1915.

*Fig. 1.*



*Fig. 2.*



*Fig. 3.*



WITNESSES:

*Mae Hofmann*  
*Howard J. O'Keig*

INVENTOR:

*Robert G. Miller*  
BY *John Wardale*

ATTORNEY:

# UNITED STATES PATENT OFFICE.

ROBERT GRIFFEN MILLER, OF MOUNT HOLLY SPRINGS, PENNSYLVANIA.

## VITREOUS WARE AND METAL AND METHOD OF MAKING SAME.

1,164,840.

Specification of Letters Patent.

Patented Dec. 21, 1915.

Application filed April 12, 1911. Serial No. 620,600.

To all whom it may concern:

Be it known that I, ROBERT GRIFFEN MILLER, a citizen of the United States, residing at Mount Holly Springs, in the county of 5 Cumberland, State of Pennsylvania, have invented a new and useful Vitreous Ware and Metal and Method of Making Same, of which the following is a specification:

My invention relates to structures combining vitreous ware and metal.

My object is to combine with a vitreous ware an alloy having heat resisting qualities, while the vitreous substance is in the plastic state and then burn the vitreous ware with 15 the metal or portion thereof embedded therein. The heat required to burn the vitreous body will not injuriously affect the metal alloy. The fusing point of the alloy is approximately 2,900° F., and the range of 20 temperature within which it would be injuriously affected is between 2,700° F. and 2,900° F., while the heat required for burning the vitreous body is approximately 2,400° F. This leaves a margin of safety 25 for the alloy of about 300° F. It is well known that the temperature at which the ordinary metals such as iron or steel would be injuriously affected is much below 2,400° F. By forming an alloy however, that will 30 stand a temperature without damage, of several hundred degrees above that necessary for burning vitreous ware I am able to combine the metal with the vitreous ware. That is, the metal or a portion thereof is embedded 35 in vitreous ware while the latter is in the plastic state so that when the same is burned the metal alloy is entirely uninjured.

It is obvious that metal parts may be advantageously combined with vitreous ware 40 for many purposes, for instance as a reinforcement for china receptacles, or as means for attaching other bodies thereto, such as an element of a hinge for a lid, or a pipe for a lavatory, or as an element for a support for 45 various operating mechanisms, and my invention is especially useful for sanitary structures or structures relating to the electric art where insulation is a requirement.

Referring to the drawings merely as examples of applications of my invention, Figure 1 is an elevation in part section of the sanitary device showing a hinge element and also a supply pipe, secured in place before burning. Fig. 2 is a part sectional view of a

combination of an electric conductor and an 55 insulating covering therefor and a metallic casing surrounding same. Fig. 3 is a sectional view of an electric switch embodying my invention.

Similar numerals refer to similar parts 60 throughout the several views.

By a careful and thorough mixture of certain base metals when in the molten state, I am able to produce an extremely cheap alloy 65 which is capable of being worked or wrought in any of the ways practically that iron or steel may be worked that is, it may be forged or cast or cut, and also it possesses a high degree of conductivity for electric currents.

In molding a sanitary device such as is 70 shown in Fig. 1, it is only necessary to mold the vitreous ware while in the plastic state into its proper form with the parts 4 and 5 of the metal alloy embedded in said vitreous ware. When the vitreous body 6 has become 75 sufficiently dry as in the ordinary treatment of china and other pottery, the same is placed in the kiln in the usual way and burnt, the heat to which the china or vitreous body is subjected as above stated, is several hundred 80 degrees below the fusing point of the metal alloy and therefore the metal parts are entirely unaffected by said burning.

In a similar way an electric conductor 7 composed of the metal alloy may be in- 85 cased in a tube 8 of vitreous material such as china, while the same is in the plastic state, and this tube again may be placed or inserted in a surrounding tube 9 of the metal alloy to form a protecting armor for said 90 insulating tube 8 of china. The whole may then be burnt in the usual way in the kiln at the temperature to which vitreous ware is usually subjected without in any way injuring the conducting member 7 of metal 95 alloy and the protecting covering 9 of metal alloy.

In a similar way the terminals 10 and 11 of the metallic alloy may be embedded in the base 12 of vitreous material when in the 100 plastic state, the whole may be burnt in the usual way in a kiln without injuriously affecting the metallic terminals.

A suitable alloy for carrying out my invention comprises 65% nickel, 22% manganese 105 and 13% iron. This forms an alloy of heat resisting characteristics above described. It will be obvious however to metallurgists that

this formula may be somewhat varied, or other ingredients added, to meet different requirements.

- A number of vitreous substances or clays 5 are suitable for combining with this alloy. For example, ordinary kaolin or china clay is a suitable substance. With this clay it is usual to combine other ingredients, such as flint, to prevent undue shrinking and feldspar 10 as a flux to meet required conditions as is well known in the pottery art. When such alloy and clay combined are subjected to heat, the expansion of the metal and the clay up to red heat, say from 600° to 800°, 15 is substantially the same. From 800° to 2,400° there is no further expansion either of metal or clay. There is a slight contraction of the clay due to escaping moisture and volatile substances. As the body cools 20 the clay and metal form a coherent and practically integral mass.

It will be obvious that the above are merely instances of an almost unlimited application of the combination of a metal alloy 25 having a high temperature point of fusion, with a vitreous body while the latter is in the plastic state and then subjecting the vitreous body to the usual temperature in burning the same without affecting injuriously the metal.

Applicant is aware that spark plugs have been manufactured by combining platinum points with a vitreous body and other combinations of enamel and the precious metals 35 have been employed, but it will be obvious that, due to the high cost of the precious metals their application to the uses and purposes herein specified are prohibited.

What I claim is:—

- 40 1. The method which consists in combining with a vitreous mass in the plastic state, a body of metal alloy having a co-efficient of expansion and contraction, corresponding substantially to that of the vitreous substance 45 and capable of withstanding, without injury, the burning heat of the vitreous mass, the body of metal alloy wholly or

partly embedded in the vitreous mass, and the combined mass then subjected to a burning heat to harden the vitreous substance. 50

2. The method which consists in combining with a plastic mass of vitreous substance, an element of alloy of nickel, and subjecting the combined mass to a degree of heat sufficient to burn the plastic mass 55 but insufficient to injure the metal element.

3. The method which consists in combining with a plastic mass of vitreous substance, an element comprising substantially 65% nickel, 22% manganese and 13% iron, 60 and subjecting the combined mass to a degree of heat sufficient to burn the plastic mass but insufficient to injure the metal element.

4. A body of vitreous substance and a 65 body of metal alloy, having a co-efficient of expansion corresponding substantially to that of the vitreous substance, combined therewith, the vitreous substance burned hard about the metal body and the two 70 bodies comprising a rigid coherent mass.

5. A body of burned vitreous substance and an element of alloy of nickel combined therewith, the vitreous body and the metal element comprising a rigid coherent mass. 75

6. A body of burned vitreous substance and an element comprising substantially 65% nickel, 22% manganese and 13% iron combined therewith in a rigid coherent mass.

7. In a body of china clay and a body of 80 metal alloy of the character described combined therewith, the china clay burned hard about the metal body and the two bodies comprising a rigid coherent mass.

8. The method which consists in combining a body of metal alloy of the character described with a mass of china clay in the plastic state and hardening the plastic mass by burning. 85

ROBERT GRIFFEN MILLER.

Witnesses:

MAE HOFFMANN,  
HOWARD T. OKIE.